

May 16, 1933.

A. B. PÖSCHEL

1,909,631

ORNAMENTATION

Filed Dec. 7, 1931

*Fig. 1*



*Fig. 2*



*Fig. 3*



*Fig. 4*



*Fig. 5*



INVENTOR

Alfred B. Poschel  
BY  
Augustus M. Henry  
ATTORNEY

## UNITED STATES PATENT OFFICE

ALFRED B. FÖSCHEL, OF BROOKLYN, NEW YORK

## ORNAMENTATION

Application filed December 7, 1931. Serial No. 579,361.

This invention relates to the decoration or other marking of a desired base material, by heat and pressure transfer, that is, by employing heat and pressure to transfer to said base material decorative or other matter previously printed in a pigmented ink or inks upon a temporary paper carrier, with such ink dried preparatory to the transfer step. In ordinary transfer work of this kind, the use of such a printed and dried transfer sheet has necessitated the expenditure of costly time and labor for the moistening and removing of the paper carrier; after the printed face of the latter has been laid down against the surface of the base material to be decorated, and after the thus stacked elements have been subjected to heat and pressure to effect the transfer.

One of the principal objects of the present invention is to provide a new and valuable method of fabricating a transfer sheet printed with pigmented inks and of effecting a transfer of such printed matter to a selected base material, whereby after the heat and pressure transfer the paper carrier may be stripped off immediately and without preliminary wetting.

Another important object of the present invention is to provide a method of the kind just indicated, wherein the paper carrier may act not only as the usual temporary carrier of the printed matter but also as the direct support therefor; whereby there is provided as a new article of manufacture, a transfer sheet comprising merely a paper carrier, and matter printed directly thereon, as distinguished from previous transfer sheets comprising said paper carrier, a layer of a special material spread over said carrier to provide a coat of measureable thickness, and a pattern or design printed on said layer.

The present invention differs from that disclosed in my co-pending application Serial No. 560,245, since the latter relates to the transfer of dyes or dye-including inks; although after the transfer of the dye or dye-including material, dry-stripping of the paper carrier is possible. The present invention further differs from my said co-pending application, since the latter employs a trans-

fer sheet including a layer of special material between the paper carrier and the applied matter to be transferred,—said special material proposed by my said co-pending application, however, being non-water-soluble material, whereas the special material of the art prior thereto has been water-soluble material, such as gum arabic, starch or the like.

The purpose of said layer of said special material is to support the applied ink or dye, and at the same time protect the same against absorption by the paper carrier. According to the present invention, such absorption is prevented, or avoided to other than a negligible extent, yet no special coating of the paper carrier is required.

The invention thus provides a simplified and highly economical transfer method for the decoration or marking of a selected base material; successful results having been had even with such a fibrous base material as leather.

The invention will be more clearly understood from the following description, when taken in connection with the accompanying drawing, in which:

Fig. 1 is a fragmentary elevation showing a portion of the paper carrier, and indicating a treatment thereof preparatory to the addition of printing thereto to form the new transfer sheet;

Fig. 2 is a similar view showing the completed transfer sheet;

Fig. 3 is a similar view showing a base material, and indicating a treatment thereof preparatory to the transfer step;

Fig. 4 is a fragmentary perspective view partially broken away and partially in section, showing the elements of Figs. 2 and 3 stacked in preparation for subjection to heat and pressure to perform the transfer step; and

Fig. 5 shows the stack of Fig. 3 in a press adapted to apply the heat and pressure.

It will be understood that these graphic showings are illustrative only, and are given to meet the requirement that the invention be thus graphically illustrated. It is also pointed out that these views are wholly diagrammatic, with certain thicknesses exag-

gerated, and with no attempt made to indicate relative thicknesses.

Referring to Fig. 1 more in detail, a suitable paper sheet is first impregnated, as by means of immersion or spraying, with a material to act as an ink-absorption minimizer and ink softener. This material is a liquid mixture including one or more volatile solvents, one or more oils, fats or waxes, and 10 phenol. Various formulæ have in practice been found satisfactory. A recommended formula is the following:—

|                 |           |
|-----------------|-----------|
| Toluol          | 6 gallons |
| Kerosene oil    | 2 gallons |
| Neat's foot oil | 2 gallons |
| Phenol          | 7 pounds  |

Another formula giving good results is the following:—

|                      |               |
|----------------------|---------------|
| Ethylene dichloride  | 5 1/4 gallons |
| Carbon tetrachloride | 1 3/4 gallons |
| Petroleum jelly      | 14 pounds     |
| Phenol               | 7 pounds      |

After the paper is impregnated, the volatile solvents should be completely or substantially completely evaporated; it being recommended that the impregnated paper be allowed to season for from one to several 20 days. The phenol left in the paper is for the purpose of acting later, at the time of heat and pressure transfer, as a dissolving or softening agent for the pigmented ink laid down on the paper at the time the paper is 30 printed to form the new transfer sheet. The oily or greasy material remaining in the paper after the evaporation of the volatile solvents restrains such ink against other than 40 minute absorption by or penetration into the paper.

The paper selected is preferably fairly smooth to accept good clean printing; but such paper is not necessarily heavily sized or calendered or otherwise specially finished.

Referring to Fig. 2 more in detail, the printing may be executed with ordinary printing equipment and by any of the usual printing methods; for instance, lithography, typography or rotogravure may be successfully employed. However, in order to secure best results, the printing inks used should be somewhat different from those of customary composition. Ordinary printing inks include oil varnish, which will dry within a relatively short time, forming a considerable bond with the fibers of the paper; and consequently these inks are not of maximum efficiency in carrying out the present invention. Instead there is recommended an ink having a richly pigmented content; preferably so rich as to give a stiff paste were not some slow evaporating solvent incorporated.

According to the invention, the ink is thus richly pigmented, and yet is brought down 65 to the proper consistency, that is, the usual

consistency of an oil varnish printing ink by the addition of such a solvent as benzyl alcohol or ethylene glycol monomethyl ether. Such ink may be conveniently made up of the following:—

|                     | Pounds |
|---------------------|--------|
| Color pigment       | 3      |
| Linseed oil varnish | 4      |
| Copal resin         | 1/2    |
| Dibutyl phthalate   | 1      |
| Benzyl alcohol      | 1/2    |

70

80

|                                  | Pounds |
|----------------------------------|--------|
| Color pigment                    | 3      |
| Blown castor oil                 | 5      |
| Cumarone resin                   | 1/2    |
| Ethylene glycol monomethyl ether | 1 1/2  |

85

In making the ink, thorough grinding is important if not essential. Best results are obtained when the printing is so executed that neither too much nor too little ink is supplied. The feeding of the ink should be so regulated that the solids of the design will have a good ink coverage, but there should not be supplied surplus beyond this to such an extent that smearing of the half-tones of the design will occur.

After the paper is printed, the solvent content of the ink slowly evaporates, allowing the remainder of the ink to set but without drying completely from the top surface of the printing down to the paper. The ink remains thus only partially dry apparently for an indefinite period. The richly pigmented ink residue left on the paper as a result of the printing operation is only loosely connected with the fibers of the paper, and if pressure or friction is applied, the deposited ink may have a large portion thereof easily removed, but not so easily as to be capable of being accidentally smudged by lightly slipping friction such as might occur in ordinary transport and handling. In other words, said richly pigmented ink residue remains somewhat soft, yet has a certain toughness and pliability, or self-sustaining quality; which result is obtained by the addition of a proper amount of resinous material, such, for instance, as specified in the ink formulæ given.

Referring to Fig. 3 more in detail, the base material is desirably, if not essentially, treated in such manner as to carry an ink-transfer accelerator at the time of heat and pressure transfer. While the phenol residue in the paper is activated by the heat of the transfer step to soften the ink, the accelerator acts to intensify such softening. Thus the accelerator acts in conjunction with the phenol residue in the paper, thereby to hasten transfer of the ink to the base material. The accelerator, further, acts as a binder to hold the transferred ink on the base material—yet without

90

95

100

105

110

115

120

125

130

any undesirable binding action on or adhesive cling to the paper of the transfer sheet.

The practical value of this ink-transfer accelerator will be appreciated, when it is explained that a fair transfer may be occasionally effected pursuant to the invention even when the ink used for the printing of the transfer sheet is ordinary printing ink rather than a special ink as hereinabove described.

It is recommended, however, that such special ink be employed in every case; since always in transfer work the very finest possible results, and as uniform results as possible, are desirable.

If the transfer is to be made to a plain base material, or one not previously lacquered, said ink-transfer accelerator may comprise, I have found, a solution of phenol in a volatile solvent or solvents. The base material is sprayed or otherwise-coated with such solution, and while such coating is still moist, the printed face of the transfer sheet is laid against the coated side of the base material (as shown in Fig. 4), and the heat and pressure transfer effected. Thus, at the time of heat and pressure transfer, the phenol and its still unevaporated solvents on the base material, are applied to and squeezed under pressure and in the presence of heat (as by the press shown in Fig. 5) against the printing of the transfer sheet and against the paper carrier,—this carrier having, as aforesaid, not only a phenol content, but also a residue of oily or greasy matter. A recommended formula for said solution is the following:

|                |            |
|----------------|------------|
| Toluol         | 6½ gallons |
| Benzyl alcohol | 2½ gallons |
| Phenol         | 7 pounds   |

Another formula for said solution giving good results is the following:

|                      |           |
|----------------------|-----------|
| Ethylene dichloride  | 6 gallons |
| Carbon tetrachloride | 2 gallons |
| Benzol               | 2 gallons |
| Phenol               | 7 pounds  |

If the transfer is to be made to a base material previously coated with a pigmented or clear lacquer (for instance, nitrocellulose lacquer), the ink transfer accelerator to be carried by the base material may be provided by modifying said lacquer. Excellent results in this connection are obtained when a surplus of oil, as castor oil, is added to the lacquer. Such surplus oil content of the lacquer, at the time of the heat and pressure transfer is liberated and driven out of the heated lacquer coating, and is taken up and absorbed by the paper carrier and the ink thereon. This surplus oil is similarly liberated and similarly acts, when, as is preferred, the lacquer coating is dried before the transfer; the surplus oil in this case being liberated as soon as the lacquer coating becomes thermoplasticized.

The liberated oil acts, in conjunction with the phenol residue in the paper, as an ink-transfer accelerator pursuant to the invention. That is to say, this liberated oil acts to intensify the softening action of the phenol in the paper carrier on the ink of the latter, in the presence of the heat of the transfer; so that, here also, a perfect transfer is effected.

Further, in the case of a lacquered base material, the surplus oil in such lacquer serves another useful purpose as will now be explained. Many ordinary commercial lacquers, when used as a base coating for a base material, have a tendency, as the result of a heat and pressure transfer, to stick to the paper carrier of the transfer sheet and thereby make removal of the latter difficult if not impossible. I have found that when an ordinary commercial lacquer has a surplus oil content pursuant to the invention, this sticking trouble is completely overcome.

A recommended formula for the new lacquer is the following:

|                |            |
|----------------|------------|
| Butyl acetate  | 6 gallons  |
| Toluol         | 3½ gallons |
| Camphor        | 8 ounces   |
| Soluble cotton | 50 ounces  |
| Castor oil     | 1 gallon   |

Another satisfactory lacquer formula is the following:

|                     |            |
|---------------------|------------|
| Ethyl acetate       | 4½ gallons |
| Ethyl lactate       | 1½ gallons |
| Ethylene dichloride | 3 gallons  |
| Cellulose acetate   | 75 ounces  |
| Castor oil          | ½ gallon   |
| Tricresyl phosphate | ½ gallon   |

Referring to Fig. 4 more in detail, the selected base material is shown as having its coating uppermost, and the transfer sheet is shown as inverted relative to Fig. 2, so that its printing is laid down against said coating.

Referring to Fig. 5 more in detail, the stacked elements of Fig. 4 are placed in a suitable press, as one hydraulically operated; the required heat being supplied in any suitable way, preferably by heating the platen, as indicated in Fig. 5. Excellent results are obtained when the heat and pressure are applied for about from five to ten seconds; the applied temperature is about 200° F. and the pressure is about 100 lbs. per square inch.

On removal of the stack from the press, the paper sheet may be immediately stripped off by manual pull without the use of water or solvents, easily, and without blurring or smudging the transferred printing. Then the base material may be finished in any desired way, as by applying a coating of lacquer or the like, thereby to set the transferred ink.

What is claimed is:

1. A transfer sheet comprising a paper

sheet carrying phenol and an oleaginous material, and a marking printed thereon.

2. A transfer sheet comprising a paper sheet carrying phenol and an oleaginous material, and a marking printed thereon in non-setting ink.

3. The method of marking a selected base material by transfer, which involves printing a marking on a paper sheet containing an oleaginous material, applying a coating including phenol to said base material, and effecting the transfer of said marking to said base material by heat and pressure.

4. The method of marking a selected base material by transfer, which involves printing a marking on a paper sheet containing phenol, applying a coating including an oleaginous substance to said base material, and effecting the transfer of said marking to said base material by heat and pressure.

5. The method of marking a selected base material by transfer, which involves printing a marking on a paper sheet containing phenol and an oleaginous substance, applying a coating including phenol to said base material, and effecting the transfer of said marking to said base material by heat and pressure.

6. The method of marking a selected base material by transfer, which involves printing a marking on a paper sheet containing phenol and an oleaginous substance, applying a coating including phenol and a solvent to said base material, and effecting a transfer of said marking to said base material by heat and pressure while said coating is still moist.

7. A transfer sheet comprising a paper sheet having phenol and an oleaginous material therein, and a marking printed directly on said paper sheet in richly pigmented ink containing a slow evaporating solvent.

8. The method of preparing a transfer sheet which involves impregnating a paper sheet with a phenol solution having a volatile solvent, seasoning said paper sheet by evaporation of said solvent, and then printing directly on said sheet with an ink containing a slow evaporating solvent.

Signed at Brooklyn, in the county of Kings and State of New York this 5th day of December A. D. 1931.

ALFRED B. PÖSCHEL.